

## UNITED STATES PATENT OFFICE

2,618,556

## PROCESS FOR PREPARING PHOTOGRAPHIC EMULSIONS

Edward H. Hewitson and James A. McClintock,  
Rochester, N. Y., assignors to Eastman Kodak  
Company, Rochester, N. Y., a corporation of  
New Jersey

No Drawing. Application November 19, 1947,  
Serial No. 787,028

11 Claims. (Cl. 95—7)

1

This invention relates to a process for preparing photographic emulsions and more particularly to a process for preparing photographic silver halide emulsions.

For many years, washed gelatino-silver-halide photographic emulsions have been prepared by a process consisting of the following general steps:

(1) Preparation of a silver halide in a water-solution of gelatin by mixing a water-solution of a water-soluble silver salt (usually silver nitrate) with a water solution of a water-soluble halide (usually an ammonium halide or a halide of an alkali metal). The gelatin may be dissolved in either or both of these solutions, or in a separate solution.

(2) After the silver halide has been formed, the emulsion is digested, to a greater or lesser extent, in the presence or absence of other chemicals, to produce the desired grain size, grain size distribution, and grain sensitivity.

(3) The emulsion is then chilled and allowed to gel. More gelatin may be added before chilling, if necessary to raise the gelatin concentration so that the emulsion may be "set" to form a jelly.

(4) The gel is ground, shredded, or otherwise subdivided and the water-soluble salts are leached out by washing in water, at a temperature sufficiently low to prevent melting of the gel.

(5) When the washing is completed, the water is drained off.

(6) The washed emulsion is melted, more gelatin and other chemicals may be added to condition further the silver halide grains to produce the desired characteristics during further digestion at more or less elevated temperatures.

In preparing photographic emulsions in accordance with the above general procedure, steps (3), (4) and (5) (the chilling and "setting," the washing and the draining operations) are relatively slow, time-consuming operations. Furthermore, as the size of the batches of emulsion are increased, the time required for these operations increases, and hence the equipment and space requirements increase more than proportionately.

We have now found a process for preparing photographic silver halide emulsions which eliminates the above step (3), i. e. the chilling and "setting" step, and reduces substantially the time required for steps (4) and (5), i. e. the washing and draining steps.

It is, accordingly, an object of our invention to provide a new process for preparing photographic

10

15

20

25

30

35

40

45

50

55

2

emulsions. Other objects will become apparent hereinafter.

In accordance with our invention, we add to a photographic silver halide emulsion which contains the water-soluble salts generated during the formation of the silver halide emulsion from a water-soluble silver salt and a water-soluble halide, a water-soluble salt selected from the group consisting of ammonium salts, salts of the alkali metals having an atomic weight less than 140, and salts of metals of group II of the periodic arrangement of elements having an atomic weight of less than 140, in quantity sufficient to coagulate the silver halide, and also add to the emulsion a water-soluble acid capable of lowering the pH of the emulsion to at least 4, in quantity sufficient to lower the pH of the emulsion to at least 6, whereupon the silver halide settles out rapidly and can be readily separated from the liquid portion of the mixture, washed and redispersed to give an emulsion. The process can be carried out at any convenient temperature, advantageously from 75 to 110° F., in the case of gelatino-silver-halide emulsions. The salt or the acid may be added to the emulsion first or the salt and acid can be added simultaneously.

Our invention can be illustrated in greater detail by the following steps:

(a) A silver halide is prepared in an aqueous solution of a colloid, such as gelatin, by mixing an aqueous solution of a water-soluble silver salt (e. g. silver nitrate) with an aqueous solution of a water-soluble halide (usually an ammonium halide or a halide of an alkali metal). The colloid can be dissolved in either or both of these solutions, or in a separate solution.

(b) After the silver halide has been formed, the emulsion is digested, to a greater or lesser extent, in the presence or absence of other chemicals, to produce the desired grain size, grain size distribution and grain sensitivity.

(Thus far, our new process parallels the prior art process discussed above. At this point, however, we proceed differently from the above prior art process).

(c) An acid which is capable of lowering the pH of the emulsion to at least 4 and a coagulating or a flocculating agent for the silver halide is added to the emulsion, so that the silver halide grains clump together and settle rapidly to the bottom of the container, leaving a clear or nearly clear solution above.

At this point acknowledgement is made of the prior art process which discloses the addition to a gelatino-silver-halide emulsion of salts of metals of group IV of the periodic table, e. g. salts of lead, titanium, thorium, zirconium, etc. to coagulate the gelatin of the emulsion. When such salts containing tri- or tetravalent cations are added to the emulsion the gelatin is coagulated and the coagulated gelatin carries down the silver halide. However, the salts containing the tri- or tetravalent cation act on the gelatin to harden it permanently, thereby rendering resuspension of the silver halide very difficult. Our process differs from the aforesaid process in that it is carried out at a pH of 6 or lower, and the ammonium salts and the salts of the alkali metals and the salts of metals of group II of the periodic table having an atomic weight of less than 140, coagulate the silver halide itself rather than the gelatin, although when operating our process at a pH near the isoelectric point of the gelatin in a gelatino-silver-halide emulsion some of the gelatin is coagulated but not permanently hardened.

Following coagulation, in accordance with our invention, we proceed as follows:

- (d) Decant the supernatant liquor.
- (e) Add water (with or without a coagulating or flocculating agent) and agitate the silver halide grains to allow more of the soluble salts to be leached out, followed by settling, followed by decantation of the supernatant liquid again. (d) and (e) can be repeated as often as necessary to reduce the soluble salts to the desired concentration.
- (f) After draining the aqueous liquor from the silver halide grains, water and gelatin are added to the grains, and the grains resuspended by dissolving the gelatin, usually with heating.
- (g) The resulting emulsion is digested at more or less elevated temperature, with or without the addition of further gelatin and other chemicals, to produce the desired characteristics.

The following examples will serve to illustrate further the manner of practicing our invention. These examples illustrate our new process as applied to a "good positive emulsion" formula published in "Photographic Emulsions" by Wall, 1929 edition, page 86.

#### Example 1

|                    |            |
|--------------------|------------|
| "Potassium bromide | 460 grams  |
| Potassium iodide   | 1.04 grams |
| Hydrochloric acid  | .35 cc.    |
| Water              | 3000 cc.   |

"Temperature 50° C. (122° F.)

|                |           |
|----------------|-----------|
| Silver nitrate | 500 grams |
| Water          | 3000 cc.  |

"Temperature 50° C. (122° F.)

|          |           |
|----------|-----------|
| Gelatine | 150 grams |
| Water    | 1200 cc.  |

"Temperature 50° C. (122° F.). Run the bromide and the silver into the gelatine solution simultaneously, keeping the bromide in excess. As soon as mixed add:

|         |        |
|---------|--------|
| Ammonia | 60 cc. |
|---------|--------|

"Digest for one hour at 43° C. (110° F.) . . ."

At this point, we deviated from Wall's Formula and cooled the emulsion to approximately 100° F. Then sulfuric acid was added to lower the pH of the emulsion below 3. 400 grams of sodium

chloride were then added in the dry state. The resulting mixture was stirred until the sodium chloride dissolved, whereupon the mixture was cooled to about 70° F. The silver halide grains settled rapidly out of suspension. The supernatant liquor was then decanted and cool water (at about 60° F.) was added to make the total volume up to about twice the original volume of the uncoagulated emulsion. The mixture was then stirred briefly, the silver halide grains allowed to settle, and the supernatant liquor was decanted. This "washing process" was repeated three times, each time adding enough water to make the total volume up to about twice the original volume of uncoagulated emulsion. After the final decantation, enough water was added to make the volume up to a volume equaling the original emulsion volume.

At this point, we returned to Wall's Formula and added the following materials to the emulsion:

- "Gelatine, dry ----- 960 grams
- Ethyl alcohol ----- 650 cc.
- Chrome alum ----- 4 grams"
- (The two quantities of gelatin—730 grams added before washing and 230 grams added after washing in Wall's Formula are combined to make the 960 grams designated above).
- The total bulk was then made up to 12,500 grams with water and the resulting emulsion digested (ripened) in the usual manner.

#### Example 2

- An emulsion was prepared exactly as in Example 1, except that hydrochloric acid instead of sulfuric acid was employed to lower the pH of the emulsion to at least 3.

#### Example 3

- An emulsion was prepared exactly as in Example 1, except that hydrochloric acid was employed instead of sulfuric acid to lower the pH of the emulsion to at least 3 and 650 grams of zinc sulfate was employed instead of sodium chloride to coagulate the silver halide.

#### Example 4

- An emulsion was prepared exactly as in Example 1, except that after the decantation of the supernatant liquor from the first settling operation, 50 grams of dry sodium sulfate (anhydrous) was added. This addition helps to prevent resuspension of the silver halide grains during subsequent washing.

#### Example 5

- An emulsion was prepared exactly as in Example 1, except that 500 grams of ammonium sulfate was employed instead of sodium chloride to coagulate the silver halide.

#### Example 6

- An emulsion was prepared exactly as in Example 1, except that sulfuric acid was employed to lower the pH of the emulsion to 5 followed by citric acid to lower the pH of the emulsion to 3, and 460 grams of ammonium sulfate was employed instead of sodium chloride to coagulate the silver halide.

In the foregoing examples water-soluble halides other than potassium bromide and potassium iodide can be used, e. g. potassium chloride, sodium bromide, sodium iodide, ammonium bromide, ammonium iodide, methylammonium bro-

amide, lithium bromide, etc. Water-soluble silver salts other than silver nitrate can be used.

Many other acids can be employed to lower the pH of the emulsion to at least 6, e. g. citric, acetic, phosphoric, perchloric, etc. One or more acids can be employed. Sulfuric acid and citric acid are advantageously employed together. Many other salts can be employed to coagulate the silver halide grains. The following salts are exemplary:

|                        |                        |
|------------------------|------------------------|
| Ammonium bromide       | Potassium ferricyanide |
| Ammonium chloride      | Potassium sulfate      |
| Ammonium phosphate     | Potassium chromate     |
| Ammonium sulfate       | Potassium chloride     |
| Ammonium molybdate     | Sodium sulfate         |
| Ammonium nitrate       | Sodium chloride        |
| Barium chloride        | Sodium tetraborate     |
| Barium nitrate         | Sodium acetate         |
| Calcium chloride       | Trisodium phosphate    |
| Calcium nitrate        | Zinc chloride          |
| Magnesium sulfate      | Zinc sulfate           |
| Potassium persulfate   | Zinc nitrate           |
| Potassium ferrocyanide | Zinc bromide           |

Salts containing monovalent cations are advantageously employed. One or more salts can be employed.

Many modifications of the procedure described above can also be employed. For example, the salt can be added to the emulsion before the pH is lowered by the addition of the acids. More or less digestion time may be given before adding the acid and salt to effect coagulation. Additional gelatin can be added before the coagulation, if desired. Temperatures may be varied within wide limits and depend more upon the emulsion characteristics desired than upon the requirements of the process. More or less washing of the coagulated silver halide grains may be employed, again depending upon the emulsion characteristics desired. Also the quantities of acids and salts employed may vary within wide limits; the optimum quantities being readily determined for each individual emulsion by making simple observations.

It should be observed that our process differs extensively from those which dehydrate the emulsion, thereby producing gelation so that the emulsion can be shredded and washed without resorting to chilling operations. Processes of this nature have been employed for many years and a number of the processes are described in the literature involving the use of dehydrating salts, such as anhydrous sodium sulfate and dehydrating solvents, such as alcohol, acetone, etc. These older dehydration processes retain most or all of the gelatin which has been added to the emulsion. In our process, a large fraction of the gelatin remains dissolved in the water and is poured off during the washing operations.

As pointed out above, the quantity of acid used to lower the pH of the emulsion can be varied within relatively wide limits. The actual pH value to be obtained depends not only upon the particular coagulating salt which is employed but also upon the quantity of the coagulating salt. The optimum quantity of acid will correspond to the quantity at which the minimum amount of coagulating salt is required. The kind of acid employed also has some effect upon the amount required and upon the optimum value of pH. Similarly, the quantity of coagulating salts can be varied within wide limits. Some salts, particularly nitrates and acetates, must be employed in relatively large quantities.

Others, notably sulfates, phosphates, and molybdates may be used in relatively small quantities. It appears that the anion in any given salt is more important in determining the effectiveness of the salt than is the cation. Some salts, for example, ammonium molybdate, can be used in amounts as low as one part per 500 parts of photographic emulsion, by weight. Others, e. g. calcium nitrate must be employed at the rate of 1 part per 5 parts of emulsion.

In addition to the advantages pointed out above, the following advantages are realized by employing our new process:

1. If desired, the entire making, washing and finishing operations ordinarily employed in emulsion making may be carried out in one container, one operation following immediately after the preceding one without delay for chilling, washing and draining.
2. The amount of equipment required for the production of the emulsion is reduced.
3. More concentrated emulsions can be produced since the coagulated emulsions settle to a more compact form, to which little or much water can be added, as desired. In the usual emulsion-making process, the maximum concentration obtainable is determined by the sensitometric characteristics required. In our new process, this is not the case.
4. The time required for the production of any given type of emulsion is reduced as is the labor required.

Any of the customarily employed washed emulsions can be prepared by our new process, e. g. silver bromide, silver bromoiodide, silver chlorobromide, silver chlorobromoiodide, silver chloride, silver chloroiodide, etc. emulsions.

What we claim as our invention and secure by Letters Patent of the United States is:

1. In a process for preparing a photographic gelatino-silver-halide emulsion, the steps which consist in (1) adding to a gelatino-silver-halide emulsion which contains the water-soluble salts generated during the formation of the silver halide from a water-soluble silver salt and a water-soluble halide, after completion of the first digestion, at least one water-soluble, inorganic salt selected from the group consisting of ammonium salts, salts of the alkali metals having an atomic weight less than 140 and salts of metals of group II of the periodic arrangement of elements having an atomic weight less than 140, in quantity sufficient to coagulate the silver halide, and also adding to the emulsion at least one water-soluble acid having an ionization constant at least that of acetic acid in quantity sufficient to lower the pH to at least 6, (2) decanting the supernatant liquor, (3) adding water to the coagulated, substantially gelatin-free silver halide, (4) agitating the mixture thus obtained, (5) settling the mixture, (6) decanting the supernatant liquor, said steps (2), (3), (4), (5) and (6) being performed successively until the concentration of the water-soluble halides is reduced to the desired level, and (7) redispersing the washed silver halide grains in an aqueous gelatin solution.
2. In a process for preparing a photographic gelatino-silver-halide emulsion, the steps which consist in (1) adding to a gelatino-silver-halide emulsion which contains the water-soluble salts generated during the formation of the silver halide from a water-soluble silver salt and a water-soluble halide, after completion of the first

digestion, sodium chloride, in quantity sufficient to coagulate the silver halide, and also adding to the emulsion hydrochloric acid in quantity sufficient to lower the pH of the emulsion to at least 6, (2) decanting the supernatant liquor, (3) adding water to the coagulated, substantially gelatin-free silver halide, (4) agitating the mixture thus obtained, (5) settling the mixture, (6) decanting the supernatant liquor, said steps (2), (3), (4), (5) and (6) being performed successively until the concentration of the water-soluble halides is reduced to the desired level, and (7) redispersing the washed silver halide grains in an aqueous gelatin solution.

3. In a process for preparing a photographic gelatino-silver-halide emulsion, the steps which consist in (1) adding to a gelatino-silver-halide emulsion which contains the water-soluble salts generated during the formation of the silver halide from a water-soluble silver salt and a water-soluble halide, after completion of the first digestion, ammonium sulfate, in quantity sufficient to coagulate the silver halide, and also adding to the emulsion sulfuric acid and citric acid in quantity sufficient to lower the pH of the emulsion to at least 6, (2) decanting the supernatant liquor, (3) adding water to the coagulated, substantially gelatin-free silver halide, (4) agitating the mixture thus obtained, (5) settling the mixture, (6) decanting the supernatant liquor, said steps (2), (3), (4), (5) and (6) being performed successively until the concentration of the water-soluble halides is reduced to the desired level, and (7) redispersing the washed silver halide grains in an aqueous gelatin solution.

4. In a process for preparing a photographic gelatino-silver-halide emulsion, the steps which consist in (1) adding to a gelatino-silver-halide emulsion which contains the water-soluble salts generated during the formation of the silver halide from a water-soluble silver salt and a water-soluble halide, after completion of the first digestion, ammonium sulfate, in quantity sufficient to coagulate the silver halide, and also adding to the emulsion sulfuric acid in quantity sufficient to lower the pH of the emulsion to at least 6, (2) decanting the supernatant liquor, (3) adding water to the coagulated, substantially gelatin-free silver halide, (4) agitating the mixture thus obtained, (5) settling the mixture, (6) decanting the supernatant liquor, said steps (2), (3), (4), (5) and (6) being performed successively until the concentration of the water-soluble halides is reduced to the desired level, and (7) redispersing the washed silver halide grains in an aqueous gelatin solution.

5. In a process for preparing a photographic gelatino-silver-halide emulsion, the steps which consist in (1) adding to a gelatino-silver-halide emulsion which contains the water-soluble salts generated during the formation of the silver halide from a water-soluble silver salt and a water-soluble halide, after completion of the first digestion, an inorganic salt of an alkali metal having an atomic weight less than 140, in quantity sufficient to coagulate the silver halide, and also adding to the emulsion a water-soluble acid having an ionization constant at least that of acetic acid in quantity sufficient to lower the pH of the emulsion to at least 6, (2) decanting the supernatant liquor, (3) adding water to the coagulated, substantially gelatin-free silver halide, (4) agitating the mixture thus obtained, (5) settling the mixture, (6) decanting the supernatant liquor, said steps (2), (3), (4), (5) and (6) being performed successively until the concentration of the water-

liquor, said steps (2), (3), (4), (5) and (6) being performed successively until the concentration of the water-soluble halides is reduced to the desired level, and (7) redispersing the washed silver halide grains in an aqueous gelatin solution.

6. In a process for preparing a photographic gelatino-silver-halide emulsion, the steps which consist in (1) adding to a gelatino-silver-halide emulsion which contains the water-soluble salts generated during the formation of the silver halide from a water-soluble salt and a water-soluble halide, after completion of the first digestion, an inorganic ammonium ( $\text{NH}_4$ ) salt in quantity sufficient to coagulate the silver halide, 10 and also adding to the emulsion a water-soluble acid having an ionization constant at least that of acetic acid in quantity sufficient to lower the pH of the emulsion to at least 6, (2) decanting the supernatant liquor, (3) adding water to the coagulated, substantially gelatin-free silver halide, (4) agitating the mixture thus obtained, (5) settling the mixture, (6) decanting the supernatant liquor, said steps (2), (3), (4), (5) and (6) being performed successively until the concentration of the water-soluble halides is reduced to the desired level, and (7) redispersing the washed silver halide grains in an aqueous gelatin solution.

7. In a process for preparing a photographic gelatino-silver-halide emulsion, the steps which consist in (1) adding to a gelatino-silver-halide emulsion which contains the water-soluble salts generated during the formation of the silver halide from silver nitrate and an alkali metal halide, after completion of the first digestion, at least one water-soluble, inorganic salt selected from the group consisting of ammonium salts, salts of the alkali metals having an atomic weight less than 140 and salts of metals of group II of the periodic arrangement of elements having an atomic weight less than 140, in quantity sufficient to coagulate the silver halide, and also adding to the emulsion at least one water-soluble acid having an ionization constant at least that of acetic acid in quantity sufficient to lower the pH to at least 6, (2) decanting the supernatant liquor, (3) adding water to the coagulated, substantially gelatin-free silver halide, (4) agitating the mixture thus obtained, (5) settling the mixture, (6) decanting the supernatant liquor, said steps (2), (3), (4), (5) and (6) being performed successively until the concentration of the water-soluble halides is reduced to the desired level, and (7) redispersing the washed silver halide grains in an aqueous gelatin solution.

8. In a process for preparing a photographic gelatino-silver-halide emulsion, the steps which consist in (1) adding to a gelatino-silver-halide emulsion which contains the water-soluble salts generated during the formation of the silver halide from silver nitrate and an alkali metal halide, after completion of the first digestion, an inorganic salt of an alkali metal having an atomic weight less than 140, in quantity sufficient to coagulate the silver halide, and also adding to the emulsion a water-soluble acid having an ionization constant at least that of acetic acid in quantity sufficient to lower the pH of the emulsion to at least 6, (2) decanting the supernatant liquor, (3) adding water to the coagulated, substantially gelatin-free silver halide, (4) agitating the mixture thus obtained, (5) settling the mixture, (6) decanting the supernatant liquor, said steps (2), (3), (4), (5) and (6) being performed successively until the concentration of the water-

soluble halides is reduced to the desired level, and (7) redispersing the washed silver halide grains in an aqueous gelatin solution.

9. In a process for preparing a photographic gelatino-silver-halide emulsion, the steps which consist in (1) adding to a gelatino-silver-halide emulsion which contains the water-soluble salts generated during the formation of the silver halide from silver nitrate and an alkali metal halide, after completion of the first digestion, sodium chloride in quantity sufficient to coagulate the silver halide, and also adding to the emulsion hydrochloric acid in quantity sufficient to lower the pH of the emulsion to at least 6, (2) decanting the supernatant liquor, (3) adding water to the coagulated, substantially gelatin-free silver halide, (4) agitating the mixture thus obtained, (5) settling the mixture, (6) decanting the supernatant liquor, said steps (2), (3), (4), (5) and (6) being performed successively until the concentration of the water-soluble halides is reduced to the desired level, and (7) redispersing the washed silver halide grains in an aqueous gelatin solution.

10. In a process for preparing a photographic gelatino-silver-halide emulsion, the steps which consists in (1) adding to a gelatino-silver-halide emulsion which contains the water-soluble salts generated during the formation of the silver halide from silver nitrate and an alkali metal halide, after completion of the first digestion, ammonium sulfate in quantity sufficient to coagulate the silver halide, and also adding to the emulsion sulfuric acid and citric acid in quantity sufficient to lower the pH of the emulsion to at least 6, (2) decanting the supernatant liquor, (3) adding water to the coagulated, substantially gelatin-free silver halide (4) agitating the mixture thus obtained, (5) settling the mixture, (6) decanting the supernatant liquor, said steps (2), (3), (4), (5) and (6) being performed successively until the concentration of the water-soluble halides is reduced to the desired level, and (7) redispersing the washed silver halide grains in an aqueous gelatin solution.

11. In a process for preparing a photographic gelatino-silver-halide emulsion, the steps which

consist in (1) adding to a gelatino-silver-halide emulsion which contains the water-soluble salts generated during the formation of the silver halide from silver nitrate and an alkali metal halide, after completion of the first digestion, ammonium sulfate in quantity sufficient to coagulate the silver halide, and also adding to the emulsion sulfuric acid in quantity sufficient to lower the pH of the emulsion to at least 6, (2) decanting the supernatant liquor, (3) adding water to the coagulated, substantially gelatin-free silver halide, (4) agitating the mixture thus obtained, (5) settling the mixture, (6) decanting the supernatant liquor, said steps (2), (3), (4), (5) and (6) being performed successively until the concentration of the water-soluble halides is reduced to the desired level, and (7) redispersing the washed silver halide grains in an aqueous gelatin solution.

EDWARD H. HEWITSON.  
JAMES A. MCCLINTOCK.

#### REFERENCES CITED

The following references are of record in the file of this patent:

#### UNITED STATES PATENTS

| Number    | Name          | Date          |
|-----------|---------------|---------------|
| 1,844,716 | Lambert       | Feb. 9, 1932  |
| 2,258,755 | Glaser        | Oct. 14, 1941 |
| 2,401,051 | Crouse et al. | May 28, 1946  |
| 2,489,341 | Waller        | Nov. 29, 1949 |

#### FOREIGN PATENTS

| Number  | Country       | Date          |
|---------|---------------|---------------|
| 585,758 | Great Britain | Feb. 24, 1947 |

#### OTHER REFERENCES

The Silver Bromide Grain of Photographic Emulsions, Trivelli and Sheppard monograph, Research Laboratory, Eastman Kodak Co., pp. 33, 36 and 39 cited.

Ausfuhrliches Handbuch der Photographie, Eder, vol. 3, part 1, 6th Complete Edition by Wentzel, 1930, pp. 92, paragraph 11, 134, footnote 2, 141, paragraph 3, and 182-184, published by Halle, William Knapp, 1930.